

April 29, 1930.

H. C. THOMPSON

1,756,889

ELECTRON DISCHARGE APPARATUS

Filed Dec. 14, 1927

Fig. 1.



Fig. 2.



Inventor:  
Harry C. Thompson,  
by *Wanda S. Scott*,  
His Attorney.

## UNITED STATES PATENT OFFICE

HARRY C. THOMPSON, OF SCHENECTADY, NEW YORK, ASSIGNOR TO GENERAL ELECTRIC COMPANY, A CORPORATION OF NEW YORK

## ELECTRON-DISCHARGE APPARATUS

Application filed December 14, 1927. Serial No. 240,044.

My present invention relates to electron discharge apparatus, and more particularly to apparatus of the type in which advantage is taken of the capabilities of an electrode to 5 emit secondary or impact electrons.

It has heretofore been proposed to operate electron discharge devices having an electron emitting cathode, and two or more other electrodes, with such circuit connections that 10 emission of impact electrons from one of the electrodes may be obtained of sufficient amount to give the device a negative resistance characteristic, thereby enabling it to be utilized efficiently as an amplifier or generator 15 of high frequency currents.

One of the objects of my invention is to provide an apparatus of the character described in which the electrode which emits impact electrons is capable of doing so more 20 effectively than those heretofore known.

Still another object of my invention is to provide an improved method for coating the surface of such an electrode so that it will be efficient as an emitter of impact electrons, and 25 its property in this respect will remain substantially unchanged over a long period of operation.

I have found that the impact emitting property of an electrode may be greatly enhanced by forming on the electrode a suitable coating of a compound of a metal having alkaline properties. It is of course necessary that a compound be chosen which will be stable during the conditions of operation 30 so that the emitting properties of the electrode will not vary materially over a long period. Among the compounds which seem the most suitable for this purpose are borates 35 and oxides. I have found that very good results may be obtained by the use of borates of potassium, lithium, sodium, barium, magnesium and oxides of barium, strontium and calcium. Some of these compounds are stable 40 when used in an evacuated receptacle, al-

though they are subject to change when exposed to the air.

In some cases it is desirable to use a compound which is reduced to a different form by the application of heat. I have also found 50 it desirable to supply to the electrode during the process of manufacture of the device the vapor of a metal having alkaline properties such as calcium or magnesium. The exact mechanism whereby improved results 55 are obtained in this case is not well established, but I have found that in some cases the effectiveness of the electrode to emit impact electrons is very greatly increased by this treatment.

The novel features which I believe to be characteristic of my invention are set forth with particularity in the appended claims. My invention itself, however, will best be understood by reference to the following description taken in connection with the accompanying drawing in which Figs. 1 and 2 show perspective views partly broken away 65 of two different forms of devices in which my invention has been incorporated with satisfactory results.

I have shown in Fig. 1 of the drawing a four-element discharge device of the so-called screen grid type. This device comprises a centrally located filamentary cathode 1 surrounded by a control grid 2. The control grid is in turn surrounded by a screening grid 3 and an anode 4 surrounds the electrodes 1, 2 and 3. The screening system is completed by an additional grid 5 which surrounds the anode and is electrically connected to the inner screening grid 3. When such a device is used for amplification purposes and a fixed positive potential is applied to the screening grid the effectiveness is somewhat reduced 75 because of the fact that a certain percentage of the electrons emitted from the cathode are absorbed by the screening grid and do not reach the anode. To overcome this disadvantage I have found that the screening grid 80

may be coated so as to emit impact electrons which pass to the anode, and if the device is operated in such a way that the impact electrons emitted are equal in number to the primary electrons reaching the screening grid then the effect of this grid in reducing the current reaching the anode may be entirely eliminated. Such a device may also be used effectively as a pliodynatron.

10 Fig. 2 shows a three-element device which may be used as a dynatron. This comprises the usual electron emitting cathode 6, grid electrode 7 surrounding the cathode and an anode or plate electrode 8 surrounding the 15 grid and cathode.

15 In the manufacture of devices such as illustrated in Figs. 1 and 2, the electrodes which are to be treated to make them efficient impact emitters, are before mounting in the 20 tube coated with the selected compound of the metal having alkaline properties. This may be done in a variety of ways; for example, if a borate is employed and the plate electrode is to be coated, a bead of the borate 25 may be formed on the grid support and this may be evaporated off into the plate by electron bombardment of the grid. Any of the borates previously mentioned may be used in this way. One borate which I have found 30 especially suitable is lithium borate. This has the advantage that electrodes treated therewith have been found to emit practically one impact electron for every primary electron reaching them at a voltage as low as 12 35 volts.

Still another method which may be used to advantage in forming a coating is to mix the coating compound with a thin varnish such as amyl-acetate-zapon varnish, applying this 40 as a very thin coating on the electrode, and permitting it to dry before mounting the electrode in the bulb. When the coating is made in this way the electrode is heated during evacuation of the device in order to fix 45 the coating in such a way as to obtain the desired emitting properties. The temperature required for this will vary somewhat with the particular compound used. It should in most cases be at least 1000° K. and should 50 not be high enough to evaporate the coating from the surface.

I have found that the emitting properties of the electrodes coated in the manner which I have described or in other ways are greatly 55 improved by supplying to the space adjacent the coated surface a metal vapor having alkaline properties, such, for example, as the vapor of magnesium or calcium. In Figs. 1 and 2, I have indicated a convenient way 60 of supplying such a vapor which consists in securing to the grid supports a quantity 9 of metal in the form of a paste. In the process of evacuation the outer electrode or plate is first heated to fix the coating thereon and this 65 heating may be carried far enough to cause

the vaporization of the metal on the grid support, thus furnishing the vapor directly to the space adjacent the coated surface while that surface is at a high temperature. Other ways of mounting the metal may be used if desired, the essential features being 70 that it is so placed that it may readily be vaporized and that the vapor will be supplied directly to the coated surface.

Some of the compounds which are effective 75 in producing a good electron emission are comparatively unstable in the air, but are stable in the inside of the evacuated receptacle after the air has been exhausted therefrom. One example of such a compound is barium oxide. To overcome this disadvantage I have found that good results may be obtained by using barium peroxide to form 80 the coating. By the subsequent heating of the coated electrode this peroxide is reduced to the oxide and good results may be obtained.

I have not as yet determined the exact reason why the use of the metal vapor enhances 90 the emitting properties of the coated surface. It appears likely that a partial reduction of the coating compound takes place which renders the coating more efficient in emitting impact electrons and that the resulting compound is less stable than the original. In 95 any event I have found that a surface which has been sensitized in the manner described loses its sensitivity if it is exposed to the air.

What I claim as new and desire to secure by Letters Patent of the United States, is:—

100 1. An electron discharge device comprising an evacuated receptacle containing an electron emitting cathode and two other electrodes, one of said other electrodes having formed thereon a coating of a lithium compound whereby the electrode thus coated is capable of serving as an efficient emitter of impact electrons.

105 2. The method of forming an efficient impact electron emitting surface on an electrode of an electron discharge device which consists in coating the surface of said electrode with a compound of a metal having alkaline properties, mounting the electrode in a receptacle, evacuating the receptacle, heating the electrode and supplying to the space adjacent the surface a vapor of a metal having 110 alkaline properties.

115 3. The method of forming an efficient impact electron emitting surface on an electrode of an electron discharge device having a cathode, an anode and a grid which consists in coating the surface of said electrode with a compound of a metal having alkaline properties, securing to the grid a quantity of a metal having alkaline properties, mounting the electrodes in a receptacle, evacuating the receptacle, and supplying sufficient heat to the anode to vaporize the metal having alkaline properties.

4. The method of forming an efficient impact electron emitting surface on an electrode of an electron discharge device having a cathode, an anode, and a grid which consists in  
5 coating the surface of said electrode with a compound of a metal having alkaline properties, mounting within the space enclosed by the electrode a quantity of a metal having alkaline properties, mounting the electrodes  
10 in a receptacle, evacuating the receptacle, and supplying sufficient heat to the anode to vaporize the metal having alkaline properties.

In witness whereof, I have hereunto set  
my hand this 13th day of December, 1927.

15 HARRY C. THOMPSON.

20

25

30

35

40

45

50

55

60

65